# EUROPEAN PATENT APPLICATION

(11) **EP 4 596 787 A1**
(43) Date of publication of application: **06.08.2025**
(21) Application number: 24862517.0
(22) Date of filing: 08.08.2024
(51) Int. Cl.: D21H 21/18, D21H 17/60

(54) **PULP COMPOSITION**

(30) Priority: 07.09.2023 JP 2023145515
(71) Applicant: DAIKIN INDUSTRIES, LTD., Osaka-shi, Osaka 530-0001 (JP)
(72) Inventor: SHIBATA, Shun, Osaka-Shi, Osaka 530-0001 (JP); AKUTA, Ryo, Osaka-Shi, Osaka 530-0001 (JP)
(74) Representative: Hoffmann Eitle
(86) International application number: PCT/JP2024/028508
(87) International publication number: WO 2025/052863

(57) **Abstract**

The present invention provides a novel pulp composition with which it is possible to produce a pulp molded article that has improved strength. The pulp composition contains pulp, wax, and a paper strengthening agent. The paper strengthening agent comprises at least one that is selected from the group consisting of a polyacrylamide-based paper strengthening agent, a polysaccharide-based paper strengthening agent, and a polyamide-based paper strengthening agent. The amount of the wax is 0.2% by weight to 10.0% by weight inclusive with respect to the pulp. The pulp composition satisfies at least one of the following requirements (1) to (3). (1) The amount of the polyacrylamide-based paper strengthening agent is 0.1% by weight to 1.1% by weight inclusive with respect to the pulp. (2) The amount of the polysaccharide-based paper strengthening agent is 0.6% by weight to 5.0% by weight inclusive with respect to the pulp. (3) The amount of the polyamide-based paper strengthening agent is 0.3% by weight to 0.9% by weight inclusive with respect to the pulp.

## Description

### Technical Field

The present disclosure relates to a wax and an oil resistant agent for pulp.

### Background Art

Patent Literature 1 discloses a colored paperboard with two or more paper layers in which a dye, a water resistant agent and a water-repellent agent are internally added to the surface layer.

### Citation List

### Patent Literature

Patent Literature 1: JP 2013-129948 A

### Summary of Invention

### Technical Problem

Patent Literature 1 does not examine the type or amount of paper strength agent used, nor does it describe or suggest the strength of pulp formed articles.

An object of the present disclosure is to provide a novel pulp composition from which a pulp formed article having improved strength can be produced.

### Solution to Problem

The present disclosure includes the following embodiments.

### [Item 1]

A pulp composition comprising pulp, a wax and a paper strength agent, wherein
the paper strength agent is at least one selected from the group consisting of a polyacrylamide paper strength agent, a polysaccharide paper strength agent and a polyamide paper strength agent,
the amount of the wax is 0.2% by weight or more and 10.0% by weight or less based on the pulp, and
the pulp composition satisfies at least one of the following (1) to (3):
   (1) an amount of the polyacrylamide paper strength agent is 0.1% by weight or more and 1.1% by weight or less based on the pulp;
   (2) an amount of the polysaccharide paper strength agent is 0.6% by weight or more and 5.0% by weight or less based on the pulp; and
   (3) an amount of the polyamide paper strength agent is 0.3% by weight or more and 0.9% by weight or less based on the pulp.

### [Item 2]

The pulp composition according to item 1, wherein the amount of the polyacrylamide paper strength agent is 0.1% by weight or more and 1.1% by weight or less based on the pulp.

### [Item 3]

The pulp composition according to item 1 or 2, wherein the amount of the polysaccharide paper strength agent is 0.6% by weight or more and 5% by weight or less based on the pulp.

### [Item 4]

The pulp composition according to any one of items 1 to 3, wherein the amount of the polyamide paper strength agent is 0.3% by weight or more and 0.9% by weight or less based on the pulp.

### [Item 5]

The pulp composition according to any one of items 1 to 4, wherein the wax is petroleum wax.

### [Item 6]

The pulp composition according to any one of items 1 to 5, wherein the wax is at least one selected from the group consisting of paraffin wax and microcrystalline wax.

### [Item 7]

The pulp composition according to any one of items 1 to 6, wherein the wax is paraffin wax.

### [Item 8]

The pulp composition according to any one of items 1 to 7, comprising at least one selected from the group consisting of benzalkonium chloride, formic acid, acetic acid and rosin.

### [Item 9]

The pulp composition according to any one of items 1 to 8, which is free of dye.

### [Item 10]

The pulp composition according to any one of items 1 to 9, wherein
the wax is paraffin wax, and
the pulp composition comprises at least one selected from the group consisting of benzalkonium chloride, formic acid, acetic acid and rosin.

### [Item 11]

A pulp formed article formed of the pulp composition according to any one of items 1 to 10.

### [Item 12]

The pulp formed article according to item 11, comprising a further wax and a further paper strength agent adhering to the surface.

### [Item 13]

The pulp formed article according to item 11 or 12, which is for food contact.

### [Item 14]

A method for producing the pulp composition according to any one of items 1 to 10, comprising:
a wax addition step of adding the wax to the pulp; and
a paper strength agent addition step of adding the paper strength agent to the pulp.

### Advantageous Effect of Invention

The present disclosure can provide a pulp formed article having improved strength.

### Description of Embodiments

The pulp composition according to the present disclosure includes a repellent component, and a pulp formed article formed of the pulp composition has not only excellent strength but also excellent liquid repellency. Furthermore, the pulp composition according to the present disclosure has excellent pulp formability. The pulp product prepared from the pulp composition according to the present disclosure also has excellent re-disintegrating properties (recyclability).

### <Repellent>

The repellent according to the present disclosure adheres to a substrate (in particular, a pulp substrate) and imparts liquid-repellency, for example, water resistance, oil resistance, water-repellency, oil-repellency and/or antifouling properties to the substrate, and may function as a water-resistant agent, an oil-resistant agent, a water-repellent agent, an oil-repellent agent and/or an antifouling agent.

The repellent according to the present disclosure may include wax as an active ingredient (the wax will be described in detail separately in {Wax}). The wax itself may be used as a repellent, or may be used as a repellent in combination with other components described below.

The repellent of the present disclosure may not include one selected from the group consisting of a compound having a fluoroalkyl group having 8 or more carbon atoms, a compound having a perfluoroalkyl group having 8 or more carbon atoms, a compound having a fluoroalkyl group having 4 or more carbon atoms, a compound having a perfluoroalkyl group having 4 or more carbon atoms, a compound having a perfluoroalkyl group, a compound having a fluoroalkyl group and a compound having a fluorine atom. The repellent of the present disclosure can impart liquid-repellency to a substrate without these fluorine compounds.

The volume abundance ratio of particles with a size of 100 µm or larger in the repellent of the present disclosure may be 0.1% or more, 0.3% or more, 0.5% or more, 1% or more, 1.5% or more, 3% or more, 4% or more, 5% or more, or 10% or more, and may be 50% or less, 30% or less, 20% or less, 15% or less, 10% or less, 5% or less, 3% or less, or 1.5% or less as measured by laser diffraction scattering. The method for setting the volume abundance ratio of particles with a size of 1 µm or larger as measured by laser diffraction scattering to the above range is not limited, and for example, particles in the raw material and/or dispersion may be formed into fine particles using a pulverizer or a homogenizer.

The repellent of the present disclosure may have a volume median diameter measured by laser diffraction scattering of 0.01 µm or more, 0.05 µm or more, 0.1 µm or more, 0.2 µm or more, 0.3 µm or more, 0.4 µm or more, 0.5 µm or more, or 0.6 µm or more, and may have a volume median diameter of 10 µm or less, 5 µm or less, 3 µm or less, 1 µm or less, 0.9 µm or less, 0.8 µm or less, 0.7 µm or less, 0.6 µm or less, 0.5 µm orless, 0.4 µm or less, 0.3 µm or less, or 0.2 µm or less, and preferably 1 µm or less. In the present disclosure, the volume median diameter refers to the median diameter (D50) in a volume-based particle size distribution by laser diffraction scattering.

The repellent of the present disclosure may have an ionic charge density of -1,000 µeq/ g or more, -800 µeq/ g or more, -600 µeq/ g or more, -500 µeq/ g or more, -400 µeq/ g or more, -250 µeq/ g or more, -100 µeq/ g or more, -50 µeq/ g or more, -25 µeq/ g or more, 0 µeq/ g or more, 1 µeq/ g or more, 25 µeq/ g or more, 50 µeq/ g or more, 100 µeq/ g or more, 200 µeq/ g or more, and preferably -600 µeq/ g or more, and for example, -400 µeq/ g or more, -200 µeq/ g or more, or -50 µeq/ g or more, and may have an ionic charge density of 5,000 µeq/ g or less, 2,500 µeq/ g or less, 1,000 µeq/ g or less, 750 µeq/ g or less, 500 µeq/ g or less, 400 µeq/ g or less, 350 µeq/ g or less, 300 µeq/ g or less, 200 µeq/ g or less, 100 µeq/ g or less, or 50 µeq/ g or less, and preferably 1,000 µeq/ g or less, more preferably 500 µeq/ g or less, and for example, 300 µeq/ g or less. The repellent of the present disclosure has an ionic charge density of preferably -600 µeq/g or more and 100 µeq/g or less. The ionic charge density of the repellent of the present disclosure may be measured by the following method.

The anion requirement of a sample aqueous solution having a solid content of 0.1 g/L is measured by a particle charge meter (MUTEK PCD-04 manufactured by BTG) using a 1/1,000 N potassium polyvinyl sulfonate solution, and the ionic charge density (cationic charge density) is calculated by the following equation (1). Alternatively, the cation requirement is measured in the same manner by using poly(diallyldimethylammonium chloride) solution instead of the potassium polyvinylsulfonate solution to calculate the ionic charge density (anionic charge density) by the following equation (1). $Ionic charge density \left(μeq/g\right) = A / B$
A: cation requirement or anion requirement (µeq/L)
B: Concentration of sample solution (g/L)

### {Wax}

The repellent according to the present disclosure may comprise a wax. The wax may be an organic material that is solid at room temperature and liquid when heated. For example, the wax may be a hydrocarbon compound or a compound having a hydrocarbon group having 6 or more and 40 or less carbon atoms (e.g., an alkyl group).

The wax in the present disclosure adheres to a substrate (in particular, a pulp substrate) and imparts liquid repellency such as water resistance, oil resistance, water-repellency, oil-repellency and/or antifouling properties to the substrate.

The wax may be a compound having a monovalent hydrocarbon group having 1 or more and 40 or less carbon atoms and optionally having a substituent or a monovalent polysiloxane group. The wax may have a hydrocarbon group having 6 or more and 40 or less carbon atoms (e.g., an alkyl group) from the viewpoint of liquid repellency.

### [Characteristics of wax]

Characteristics that the wax may have will be described below.

The wax may be in the form of particles (powder). The wax has an average particle size of 0.01 µm or more, 0.05 µm or more, 0.1 µm or more, 0.2 µm or more, 0.3 µm or more, 0.4 µm or more, 0.5 µm or more, or 0.6 µm or more, and 10 µm or less, 5 µm or less, 3 µm or less, 1 µm or less, 0.9 µm or less, 0.8 µm or less, 0.7 µm or less, 0.6 µm or less, 0.5 µm or less, 0.4 µm or less, 0.3 µm or less, or 0.2 µm or less, and preferably 1 µm or less. The above particle size is the primary particle size. The average particle size of the wax in the above range provides excellent particle stability and may improve liquid repellency. The average primary particle size may be measured by a microscope (scanning electron microscope). Specifically, a sample of wax particles is observed under a microscope at any magnification. Next, when particles are spherical, the diameter is considered as the particle size, and when particles are non-spherical, the average of the major axis and the minor axis is regarded as the particle size. By repeating measuring the particle size of all particles present in a field of view and moving to a different field of view and measuring the particle size again, 100 particle sizes or more are measured, and the average of those is defined as the average particle size.

The wax may have a HD (n-hexadecane) contact angle of 10° or more, 20° or more, 25° or more, 30° or more, 35° or more, 40° or more, 45° or more, 50° or more, 55° or more, 60° or more, or 65° or more, preferably 25° or more, and more preferably 30° or more, and 100° or less, 90° or less, or 75° or less. A HD contact angle of the wax of the lower limit or more can impart good liquid-repellency (in particular oil-repellency) to a substrate. The HD contact angle is a static contact angle of a wax to a spin-coated film, which is obtained by dropping 2 µL of HD on a spin-coated film and measuring the contact angle one second after the droplet reaches the film.

The wax may have a water contact angle of 35° or more, 40° or more, 45° or more, 50° or more, 55° or more, 65° or more, 75° or more, 85° or more, 90° or more, or 100° or more, and 160° or less, 140° or less, 130° or less, 120° or less, 110° or less, 100° or less or 90° or less. A water contact angle of the wax of the lower limit or more can impart good liquid-repellency (in particular water-repellency) to a substrate. The water contact angle is a static contact angle of a wax to a spin-coated film, which is obtained by dropping 2 µL of water on a spin-coated film and measuring the contact angle one second after the droplet reaches the film.

The wax may be a low molecular weight compound (having a weight average molecular weight of, for example, less than 1,000 or 500 or less) and/or a high molecular weight compound. When the wax is a high molecular weight compound, the wax may have a weight average molecular weight of 1,000 or more, 3,000 or more, 5,000 or more, 7,500 or more, 10,000 or more, 30,000 or more, 100,000 or more, 300,000 or more, or 500,000 or more, and 10,000,000 or less, 7,500,000 or less, 5,000,000 or less, 3,000,000 or less, 1,000,000 or less, 750,000 or less, 500,000 or less, 300,000 or less, 100,000 or less, 75,000 or less, 50,000 or less, 30,000 or less, 10,000 or less, 7,500 or less, 5,000 or less, or 3,000 or less.

The wax may have a melting point of 30°C or more, 40°C or more, 60°C or more, 80°C or more, 100°C or more, or 120°C or more, preferably 40°C or more, 50°C or more, 60°C or more, 70°C or more, or 80°C or more, and 250°C or less, 225°C or less, 200°C or less, 150°C or less, 130°C or less, 120°C or less, 110°C or less, 100°C or less, 80°C or less, or 50°C or less, and for example, 150°C or less, or 100°C or less. The melting point of wax may be measured according to JIS K 2235-1991.

### [Structure of wax]

The wax in the present disclosure may not have any one selected from the group consisting of a fluoroalkyl group having 8 or more carbon atoms, a perfluoroalkyl group having 8 or more carbon atoms, a fluoroalkyl group having 4 or more carbon atoms, a perfluoroalkyl group having 4 or more carbon atoms, a perfluoroalkyl group, a fluoroalkyl group, and a fluorine atom. The wax can impart liquid-repellency without including these fluorine-containing groups to a substrate.

The wax may be a hydrocarbon compound or a compound having a monovalent hydrocarbon group having 1 or more and 40 or less carbon atoms and optionally having a substituent or a monovalent polysiloxane group. The wax may be a hydrocarbon compound or a compound having a hydrocarbon group having 6 or more and 40 or less carbon atoms (e.g., an alkyl group) from the viewpoint of the improvement in liquid repellency.

### (Monovalent hydrocarbon group optionally having a substituent)

The wax may have a monovalent hydrocarbon group optionally having a substituent.

The hydrocarbon group may be a monovalent hydrocarbon group having 1 or more and 40 or less carbon atoms. The hydrocarbon group may be an aromatic hydrocarbon group or an aliphatic hydrocarbon group, and is preferably an aliphatic hydrocarbon group, and in particular a saturated aliphatic hydrocarbon group (an alkyl group). The hydrocarbon group may be branched, cyclic or linear, and preferably linear.

The hydrocarbon group may have 1 or more, 3 or more, 6 or more, 8 or more, 10 or more, 12 or more, 14 or more, 16 or more, 18 or more, 20 or more, or 22 or more, preferably 6 or more, 10 or more, 12 or more, or 16 or more carbon atoms, and 40 or less, 35 or less, 30 or less, 25 or less, 20 or less, 15 or less, or 10 or less, preferably 30 or less, 25 or less, or 20 or less carbon atoms.

The hydrocarbon group may have a substituent, but is preferably non-substituted. Examples of substituents include - OR', -N(R')₂, -COOR', and a halogen atom (wherein R' is independently at each occurrence a hydrogen atom or a hydrocarbon group having 1 to 30, 1 to 20, 1 to 10, or 1 to 4 carbon atoms). The substituent may or may not have active hydrogen. The number of substituents may be 6 or less, 5 or less, 4 or less, 3 or less, 2 or less, 1 or less, or 0. In the hydrocarbon group having a substituent, the amount of carbon atom relative to the carbon atom and the heteroatom may be 70 mol% or more, 80 mol% or more, 90 mol% or more, 95 mol% or more, or 99 mol% or more, and preferably 75 mol% or more, and may be 95 mol% or less, 90 mol% or less, 85 mol% or less, or 80 mol% or less. The hydrocarbon group may have 1 to 3 (for example, 1) -OR' (in particular, -OH) as a substituent (for example at a site other than the end).

### (Monovalent polysiloxane group)

The wax may have a monovalent polysiloxane group. A (monovalent) polysiloxane group can impart liquid-repellency to the substrate as the (monovalent) hydrocarbon group does.

The polysiloxane group may also be represented by the following formula:

-[-Si(R^{s})₂-O-]ₐ-

[wherein R^{s} is independently at each occurrence a hydrocarbon group having 1 to 40 carbon atoms or a reactive group, and
a is an integer of 5 or more and 10,000 or less].

R^{s} is a hydrocarbon group having 1 to 40 carbon atoms or a reactive group.

Examples of hydrocarbon groups having 1 to 40 carbon atoms include a hydrocarbon group having 1 to 5 carbon atoms and a hydrocarbon group having 6 to 40 carbon atoms.

Examples of hydrocarbon groups having 1 to 5 carbon atoms include a hydrocarbon group having 1 to 5 carbon atoms such as a methyl group, an ethyl group, a propyl group, a butyl group and a pentyl group (in particular an aliphatic hydrocarbon group, in particular an alkyl group, for example, a methyl group or an ethyl group, and in particular a methyl group).

The hydrocarbon group having 6 to 40 carbon atoms may be an aromatic hydrocarbon group or an aliphatic hydrocarbon group, and is preferably an aliphatic hydrocarbon group, and in particular a saturated aliphatic hydrocarbon group (an alkyl group). The hydrocarbon group may be cyclic, linear or branched, and preferably linear. The hydrocarbon group may have 6 or more, 8 or more, 10 or more, 12 or more, 14 or more, 16 or more, 18 or more, preferably 10 or more, more preferably 12 or more carbon atoms, and 40 or less, 35 or less, 30 or less, 25 or less, 20 or less, 15 or less, or 10 or less, preferably 30 or less, and more preferably 25 or less carbon atoms.

Examples of reactive groups include a group having a functional group (for example, a hydroxy group, an amino group, a mercapto group, an epoxy group, a carboxyl group, a halogen-substituted alkyl group, a vinyl group, a (meth)acrylic group, a (meth)acryloyloxy group, a (meth)acrylamide group, and a hydrogen atom directly bonded to a silicon atom). These functional groups may be directly bonded to a silicon atom, or may be bonded to an organic group directly bonded to a silicon atom. The organic group may be a hydrocarbon group, and for example, an alkylene group or a divalent aromatic group. The hydrocarbon group may have 2 or more and 12 or less carbon atoms. An alkylene group having 2 or more and 10 or less carbon atoms is preferred. A divalent aromatic group having 6 or more and 12 or less carbon atoms is preferred. The reactive group may be a group selected from the group consisting of a hydroxy group, an epoxy ring, a carboxyl group, a (meth)acrylic group and an amino group, and for example, may be at least one selected from the group consisting of an epoxy ring, a hydroxy group, a (meth)acrylic group and a carboxyl group.
a is 3 or more, 5 or more, 10 or more, 30 or more, 50 or more, 100 or more, 500 or more, 1,000 or more, 2,000 or more, or 3,000 or more, and preferably 10 or more, and 10,000 or less, 7,500 or less, 5,000 or less, 3,000 or less, 1,500 or less, 1,000 or less, 500 or less, 300 or less, 200 or less, 100 or less, or 50 or less, and preferably 500 or less.

In the polysiloxane group, the amount of R^{s}, which is a hydrocarbon group having 1 to 5 carbon atoms, may be 20 mol% or more, 40 mol% or more, 60 mol% or more, or 80 mol% or more, and preferably 50 mol% or more, and 100 mol% or less, 90 mol% or less, 80 mol% or less, or 70 mol% or less relative to the total amount of R^{s}. For example, 50 mol% or more of the total amount of the R^{s} group may be a methyl group or an ethyl group, and in particular, a methyl group.

In the polysiloxane group, the amount of R^{s}, which is a hydrocarbon group having 6 to 40 carbon atoms, may be 3 mol% or more, 10 mol% or more, 20 mol% or more, or 30 mol% or more, and 100 mol% or less, 90 mol% or less, 80 mol% or less, or 70 mol% or less relative to the total amount of R^{s}.

In the polysiloxane group, the amount of R^{s}, which is a reactive group, may be 5 mol% or more, 10 mol% or more, 20 mol% or more, or 30 mol% or more relative to the total amount of R^{s}, and 50 mol% or less, 40 mol% or less, 30 mol% or less, or 20 mol% or less relative to the total amount of R^{s}.

The R^{s} group may be introduced randomly or in block, and preferably randomly.

The end structure of the polysiloxane group is not limited, and may be -OR^{s}, -Si(R^{s})₃ and the like. R^{s} in the end structure may have one or more reactive groups. Examples of reactive groups are as described above, and may be at least one selected from the group consisting of an epoxy ring, a hydroxy group, a (meth)acrylic group and a carboxyl group.

The polysiloxane group may have a linker. The raw material compound and the polysiloxane group may be linked by a linker, and examples of linkers include, but are not limited to, a hydrocarbon group having 1 to 40 (for example, 1 to 20) carbon atoms optionally disconnected via an oxygen atom, and may be, for example, a (poly)oxyalkylene group having 1 to 40 (for example, 1 to 20) carbon atoms.

Examples of polysiloxane groups include

-[-Si(R^{s})₂-O-]ₐ-Si(R^{s})₃

-L^{s1}-[-Si(R^{s})₂-O-]ₐ-Si(R^{s})₃

-L^{s1}-O-L^{s1}-[-Si(R^{s})₂-O-]ₐ-R^{s}

-L^{s1}-[-Si(R^{s})₂-O-]ₐ-Si(R^{s})₃

-L^{s1}-O-L^{s1}-[-Si(R^{s})₂-O-]ₐ-R^{s}

-L^{s1}-[-Si(R^{s})₂-O-]ₐ-Si(R^{s})₃,

-L^{s1}-[-Si (R^{s})₂-O-]ₐ-R^{s}

[wherein R^{s} is independently at each occurrence a hydrocarbon group having 1 to 40 carbon atoms or a reactive group, R^{s} at the end has one or more reactive groups,
methyl groups account for 50 mol% or more of the total amount of the R^{s} group,
L^{s1} is a hydrocarbon group having 1 to 20 carbon atoms, and
a is 5 or more and 10,000 or less], and
[wherein a is an integer of 0 to 150, b is an integer of 1 to 150, (a + b) is 5 to 200 and n is an integer of 0 to 36].

### [Examples of wax]

The wax may be a hydrocarbon compound or a compound having a hydrocarbon group. Examples of hydrocarbon groups and preferred ranges are as described above. For example, the hydrocarbon group may have 6 or more and 40 or less carbon atoms.

Examples of wax include hydrocarbon wax (e.g., paraffin, polyolefin), non-hydrocarbon wax and polymer wax (e.g., vinyl polymer, silicone wax).

Examples of wax also include:
petroleum wax such as paraffin wax, microcrystalline wax, montan wax, ozokerite wax, ceresin wax and petrolatum wax; and
synthesized wax such as Fischer Tropsch wax, polyethylene wax, polypropylene wax, acrylic polymer wax, polytetrafluoroethylene wax and silicone wax.

The wax may be a hydrocarbon compound, and may not have a functional group.

### [Amount of wax]

The amount of wax may be 0.01% by weight or more, 0.5% by weight or more, 1% by weight or more, 3% by weight or more, 5% by weight or more, 10% by weight or more, 20% by weight or more, 30% by weight or more, 50% by weight or more, 70% by weight or more, or 80% by weight or more, and 95% by weight or less, 90% by weight or less, 80% by weight or less, 70% by weight or less, 60% by weight or less, 50% by weight or less, 40% by weight or less, 30% by weight or less, 20% by weight or less, 10% by weight or less, 5% by weight or less, or 3% by weight or less in the repellent. Wax may be singly used as a repellent.

### {Dispersant}

The repellent of the present disclosure may comprise a dispersant. The dispersant may be at least one selected from an organic dispersant and an inorganic dispersant. The dispersant may be at least one selected from an anionic dispersant, a nonionic dispersant, a cationic dispersant, an amphoteric dispersant and an inorganic dispersant.

An organic dispersant and an inorganic dispersant may be used as the dispersant, respectively, or an organic dispersant and an inorganic dispersant may be used in combination.

An organic dispersant may be used as the dispersant. The organic dispersant may be classified into a nonionic dispersant, an anionic dispersant, a cationic dispersant and an amphoteric dispersant. The organic dispersant may mean a surfactant.

The dispersant may have no fluorine.

### [Nonionic dispersant]

The dispersant may comprise a nonionic dispersant. The nonionic dispersant may be a nonionic surfactant.

The nonionic dispersant may be of low molecular weight or high molecular weight. The nonionic dispersant may have a molecular weight of 100 or more, 500 or more, 1,000 or more, 2,000 or more, 4,000 or more, or 6,000 or more, and 100,000 or less, 10,000 or less, 7,500 or less, 5,000 or less, 25,000 or less, 750 or less, or 250 or less.

Examples of nonionic dispersant include ether, ester, ester ether, alkanolamide, polyol and amine oxide.

The ether is, for example, a compound having an oxyalkylene group (preferably a polyoxyethylene group).

The ester is, for example, an ester of an alcohol and a fatty acid. The alcohol is, for example, an alcohol which is 1 to 30 hydric (particularly dihydric to decahydric) and has 1 to 50 carbon atoms (particularly 10 to 30 carbon atoms) (for example, an aliphatic alcohol). Examples of the fatty acids are saturated or unsaturated fatty acids having 2 to 50 carbon atoms, particularly 5 to 30 carbon atoms.

The ester ether is, for example, a compound in which an alkylene oxide (particularly ethylene oxide) is added to an ester of an alcohol and a fatty acid. The alcohol is, for example, an alcohol which is 1 to 30 hydric (particularly dihydric to decahydric) and has 1 to 50 carbon atoms (particularly 3 to 30 carbon atoms) (for example, an aliphatic alcohol). Examples of the fatty acids are saturated or unsaturated fatty acids having 2 to 50 carbon atoms, particularly 5 to 30 carbon atoms.

The alkanolamide is formed of for example, a fatty acid and an alkanolamine. The alkanolamide may be a monoalkanolamide or a dialkanolamide. Examples of the fatty acids are saturated or unsaturated fatty acids having 2 to 50 carbon atoms, particularly 5 to 30 carbon atoms. The alkanolamine may be an alkanol with 1 to 3 amino groups and 1 to 5 hydroxyl groups, having 2 to 50, particularly 5 to 30 carbon atoms.

The polyol may be, for example, a dihydric to pentahydric alcohol having 10 to 30 carbon atoms.

The amine oxide may be an oxide (for example, having 5 to 50 carbon atoms) of an amine (secondary amine or preferably tertiary amine).

The nonionic dispersant is preferably a nonionic dispersant having an oxyalkylene group (preferably a polyoxyethylene group). The alkylene group in the oxyalkylene group preferably has 2 to 10 carbon atoms. The number of oxyalkylene groups in the molecule of the nonionic dispersant is generally preferably 2 to 100.

The nonionic dispersant is selected from the group consisting of an ether, an ester, an ester ether, an alkanolamide, a polyol, or an amine oxide, and is preferably a nonionic dispersant having an oxyalkylene group.

The nonionic dispersant may be, for example, an alkylene oxide adduct of a linear and/or branched aliphatic (saturated and/or unsaturated) group, a polyalkylene glycol ester of a linear and/or branched fatty acid (saturated and/or unsaturated), a sorbitan ester of a linear and/or branched fatty acid (saturated and/or unsaturated), a glycerin ester of a linear and/or branched fatty acid (saturated and/or unsaturated), a polyglycerol ester of a linear and/or branched fatty acid (saturated and/or unsaturated), a sucrose ester of a linear and/or branched fatty acid (saturated and/or unsaturated), a polyoxyethylene (POE)/polyoxypropylene (POP) copolymer (random copolymer or block copolymer), and an alkylene oxide adduct of acetylene glycol. Among them, the nonionic dispersant is preferably a dispersant such that the structures of the alkylene oxide addition moiety and polyalkylene glycol moiety are polyoxyethylene (POE) or polyoxypropylene (POP) or POE/POP copolymer (which may be a random or block copolymer, for example.).

Furthermore, the nonionic dispersant may not include an aromatic group.

The nonionic dispersant may be the compound represented by the formula:

R¹O-(CH₂CH₂O)ₚ-(R²O)_{q}-R³

[wherein R¹ is an alkyl group having 1 to 22 carbon atoms, an alkenyl group or an acyl group, having 2 to 22 carbon atoms, R² is each independently the same or different and is an alkylene group having 3 or more carbon atoms (for example, 3 to 10),
R³ is a hydrogen atom, an alkyl group having 1 to 22 carbon atoms, or an alkenyl group having 2 to 22 carbon atoms,
p is a numeral of 2 or more,
q is 0 or a numeral of 1 or more.].

R¹ preferably has 8 to 20 carbon atoms, particularly 10 to 18 carbon atoms. Preferred examples of R¹ include an octyl group, a nonyl group, a trimethylnonyl group, a lauryl group, a tridecyl group, an oleyl group and a stearyl group.

R² is, for example, a propylene group and a butylene group.

In the nonionic dispersant, for example, p may be a numeral of 3 or more (for example, 5 to 200) and q may be a numeral of 2 or more (for example, 5 to 200). Namely, -(R²O)_{q}-may form, for example, a polyoxyalkylene chain.

The nonionic dispersant may be, for example, a polyoxyethylene alkylene alkyl ether comprising a hydrophilic polyoxyethylene chain and a hydrophobic oxyalkylene chain (particularly a polyoxyalkylene chain) in the center. The hydrophobic oxyalkylene chain includes, for example, an oxypropylene chain, an oxybutylene chain, and a styrene chain. The oxypropylene chain is preferred among them.

Specific examples of the nonionic dispersants include a condensation product of ethylene oxide with hexylphenol, isooctatylphenol, hexadecanol, oleic acid, an alkane(C₁₂-C₁₆)thiol, a sorbitan monofatty acid (C₇-C₁₉), an alkyl (C₁₂-C₁₈)amine, or the like, and a sorbitan fatty acid ester, a glycerin fatty acid ester, a polyglycerin fatty acid ester, a sucrose fatty acid ester, a propylene glycol fatty acid ester, a polyoxyethylene alkyl ether, a polyoxyethylene polyoxypropylene alkyl ether, a polyoxyethylene glycerin fatty acid ester, a polyoxyethylene sorbitan fatty acid ester, and a lecithin derivative. Examples of nonionic dispersants include polyoxyethylene alkyl ether, polyoxyethylene polyoxypropylene alkyl ether, polyoxyethylene polyoxybutylene alkyl ether, polyoxyethylene polyoxypropylene glycol and polyethyleneimine ethoxylate.

The proportion of the polyoxyethylene block can be 5 to 80% by weight, for example, 30 to 75% by weight, particularly 40 to 70% by weight, based on a molecular weight of the nonionic dispersant (copolymer).

The average molecular weight of the nonionic dispersant is generally 300 to 5,000, for example, 500 to 3,000.

For example, the nonionic dispersant may be used singly or in admixture of two or more. The nonionic dispersant may be a mixture of a compound with an HLB (hydrophilic-hydrophobic balance) of less than 15 (particularly 5 or less) and a compound with an HLB of 15 or more. More specifically, it is preferable to select the nonionic dispersant from polyoxyethylene alkyl ether, polyoxyethylene polyoxypropylene alkyl ether, polyoxyethylene and polyoxypropylene having an HLB of 1 to 18, sorbitan fatty acid ester, glycerol fatty acid ester, polyglycerol fatty acid ester, sucrose fatty acid ester, propylene glycol fatty acid ester, polyoxyethylene glycerol fatty acid ester and polyoxyethylene sorbitan fatty acid ester having an HLB of less than 7.

### [Cationic dispersant]

The dispersant may comprise a cationic dispersant. The cationic dispersant may be a cationic surfactant. The cationic dispersant may be a compound not having an amide group.

The cationic dispersant may be of low molecular weight (with a molecular weight of 2,000 or less, in particular, 10,000 or less) or of high molecular weight (with a molecular weight of, for example, 2,000 or more). The cationic dispersant may not have an amide group. The cationic dispersant may have a molecular weight of 100 or more, 500 or more, 1,000 or more, 2,000 or more, 4,000 or more, or 6,000 or more, and 1,000,000 or less, 750,000 or less, 500,000 or less, 250,000 or less, 100,000 or less, 50,000 or less, 10,000 or less, 7,500 or less, 5,000 or less, 25,000 or less, 750 or less, or 250 or less.

The cationic dispersant may be aliphatic or aromatic, and examples thereof include an ammonium salt (e.g., quaternary ammonium salt). The cationic dispersant may be oxyethylene-added ammonium salt. Specific examples thereof include an amine salt dispersant such as alkylamine salt, an amino alcohol fatty acid derivative, a polyamine fatty acid derivative and imidazoline; a quaternary ammonium salt dispersant such as alkyl trimethyl ammonium salt, dialkyl dimethyl ammonium salt, alkyl dimethyl benzyl ammonium salt, pyridinium salt, alkyl isoquinolinium salt, benzalkonium chloride and benzethonium chloride; and a polymer cationic dispersant such as polyquaternium-1 to 47. Examples of cationic dispersants include an alkylamine salt and a quaternary ammonium salt.

The low molecular weight cationic dispersant may be a compound represented by the formula:

R²¹-N⁺(-R²²)(-R²³)(-R²⁴)X⁻

wherein R²¹, R²², R²³ and R²⁴ are hydrogen or a hydrocarbon group having 1 to 40 carbon atoms, and
X is an anionic group.

Specific examples of R²¹, R²², R²³ and -R²⁴ include an alkyl group (e.g., a methyl group, a butyl group, a stearyl group, a palmityl group) and an aromatic group (e.g., a benzyl group, a phenyl group). Specific examples of X include a halogen (e.g., chlorine) and an acid (e.g., hydrochloric acid and acetic acid). The cationic dispersant may be monoalkyltrimethylammonium salt (in which alkyl has 4 to 40 carbon atoms) and benzalkonium chloride.

More specifically, the low molecular weight cationic dispersant may be an ammonium salt represented by the formula:

R¹ₚ-N⁺-R²_{q}X⁻

[wherein R¹ is a C12 or higher (e.g., C₁₂ to C₅₀) linear and/or branched aliphatic (saturated and/or unsaturated) group,
R² is H or a C1 to 4 alkyl group, a benzyl group, a polyoxyethylene group (in which the number of oxyethylene groups is for example, 1 (in particular 2, and especially 3) to 50) (particularly preferably CH₃, C₂H₅),
X is a halogen atom (e.g., chlorine) or a C₁ to C₄ fatty acid salt or a C₁ to C₄ sulfonate,
p is 1 or 2, q is 2 or 3 and p + q = 4.]
R¹ may have 12 to 50, and for example 12 to 30 carbon atoms.

Examples of the low molecular weight cationic dispersants may include dodecyltrimethylammonium acetate, trimethyltetradecylammonium chloride, hexadecyltrimethylammonium bromide, trimethyloctadecylammonium chloride, (dodecylmethylbenzyl)trimethylammonium chloride, benzyldodecyldimethylammonium chloride, methyldodecyl di(hydropolyoxyethylene) ammonium chloride, benzyldodecyl di(hydropolyoxyethylene) ammonium chloride, and N-[2-(diethylamino)ethyl]oleamide hydrochloride.

The high molecular weight cationic dispersant may be a polymer having a cationic group (for example, an ammonium group, a quaternary ammonium group) (for example, polypolyquaternium-1 to 47). Examples of high molecular weight cationic dispersants include a cationic natural product (in particular, cationic sugar) such as cationic starch, cationic cellulose (e.g., O-(2-hydroxy-3-(trimethylammonio)propyl)hydroxyethyl cellulose chloride), cationic guar gum, cationic xanthan gum and chitosan; a polymer of a cationic group-containing monomer such as aziridine, vinyl imidazole, aminoalkyl methacrylate, N,N,N',N'-tetramethyl-2-butene-1,4-diamine, quaternary dimethyl ammonium ethyl methacrylic acid, diallyldimethylammonium chloride, dimethylaminopropylamine and quaternary vinyl imidazole.

### [Anionic dispersant]

The dispersant may comprise an anionic dispersant. The anionic dispersant may be an anionic surfactant. The dispersant may not include an anionic dispersant.

The anionic dispersant may be of low molecular weight or high molecular weight. The anionic dispersant may have a molecular weight of 100 or more, 500 or more, 1,000 or more, 2,000 or more, 4,000 or more, or 6,000 or more, and 100,000 or less, 10,000 or less, 7,500 or less, 5,000 or less, 25,000 or less, 750 or less, or 250 or less.

Examples of the anionic dispersant include an alkyl ether sulfate, an alkyl sulfate, an alkenyl ether sulfate, an alkenyl sulfate, an olefin sulfonate, an alkanesulfonate, a saturated or unsaturated fatty acid salt, an alkyl or alkenyl ether carbonate, an α-sulfone fatty acid salt, a N-acylamino acid dispersant, a phosphate mono- or diester dispersant, and a sulfosuccinic acid ester. Examples of anionic dispersants include a carboxylic acid salt (e.g., fatty acid salt).

### [Amphoteric dispersant]

The dispersant may comprise an amphoteric dispersant. The amphoteric dispersant may be an amphoteric surfactant.

The amphoteric dispersant may be of low molecular weight or high molecular weight. The amphoteric dispersant may have a molecular weight of 100 or more, 500 or more, 1,000 or more, 2,000 or more, 4,000 or more, or 6,000 or more, and 100,000 or less, 10,000 or less, 7,500 or less, 5,000 or less, 25,000 or less, 750 or less, or 250 or less.

Examples of the amphoteric dispersants include, for example, alanines, imidazolinium betaines, amidobetaines, and acetic acid betaine, and specific examples of the amphoteric dispersants include, for example, lauryl betaine, stearyl betaine, lauryl carboxymethyl hydroxyethyl imidazolinium betaine, lauryl dimethylamino acetic acid betaine, and fatty acid amidopropyldimethylaminoacetic acid betaine.

### [Inorganic dispersant]

The dispersant may comprise an inorganic dispersant.

The inorganic dispersant has an average primary particle size of 5 nm or larger, 30 nm or larger, 100 nm or larger, 1 µm or larger, 10 µm or larger, or 25 µm or larger, and 100 µm or smaller, 50 µm or smaller, 10 µm or smaller, 1 µm or smaller, 500 nm or smaller, or 300 nm or smaller. The average primary particle size may be measured by a microscope, for example, a scanning electron microscope or a transmission electron microscope. The inorganic dispersant may be hydrophilic particles.

Examples of inorganic dispersants include polyvalent metal phosphate such as tricalcium phosphate, magnesium phosphate, aluminum phosphate, zinc phosphate and hydroxyapatite; carbonate such as calcium carbonate and magnesium carbonate; silicate such as calcium metasilicate; sulfate such as calcium sulfate and barium sulfate; and hydroxide such as calcium hydroxide, magnesium hydroxide and aluminum hydroxide.

### [Amount of Dispersant]

The amount of dispersant may be 0.01 parts by weight or more, 0.1 parts by weight or more, 1 part by weight or more, 3 parts by weight or more, 5 parts by weight or more, 10 parts by weight, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less 30 parts by weight or less, 20 parts by weight or less, 10 parts by weight or less, 5 parts by weight or less, 3 parts by weight or less, or 1 part by weight or less.

### {Liquid medium}

The repellent in the present disclosure may comprise a liquid medium. The liquid medium may be water, an organic solvent, or a mixture of water and an organic solvent. The repellent may be a dispersion or a solution. The repellent in the present disclosure may include at least water.

Examples of the organic solvents include esters (for example, esters having 2 to 40 carbon atoms, specifically ethyl acetate and butyl acetate), ketones (for example, ketones having 2 to 40 carbon atoms, specifically methyl ethyl ketone and diisobutyl ketone), alcohols (for example, alcohols having 1 to 40 carbon atoms, specifically isopropyl alcohol), aromatic solvents (for example, toluene and xylene), petroleum-based solvents (for example, alkanes having 5 to 10 carbon atoms, specifically, naphtha and kerosene). The organic solvent is preferably a water-soluble organic solvent. The water-soluble organic solvent may include a compound having at least one hydroxy group (for example, polyol such as alcohol and glycol solvent, and an ether form of polyol (for example, a monoether form)). These may be used alone, or two or more of them may be used in combination.

### [Amount of liquid medium]

The amount of liquid medium may be 1 part by weight or more, 3 parts by weight or more, 5 parts by weight or more, 10 parts by weight or more, 20 parts by weight or more, 30 parts by weight or more, 40 parts by weight or more, or 50 parts by weight or more, 100 parts by weight or more, 200 parts by weight or more, 300 parts by weight or more, 500 parts by weight or more, or 1,000 parts by weight or more, and 3,000 parts by weight or less, 2,000 parts by weight or less, 1,000 parts by weight or less, 500 parts by weight or less, 200 parts by weight or less, 175 parts by weight or less, 150 parts by weight or less, 125 parts by weight or less, 100 parts by weight or less, 80 parts by weight or less, 60 parts by weight or less, 40 parts by weight or less, 20 parts by weight or less, or 10 parts by weight or less relative to 1 part by weight of the wax.

The amount of water may be 1 part by weight or more, 3 parts by weight or more, 5 parts by weight or more, 10 parts by weight or more, 20 parts by weight or more, 30 parts by weight or more, 40 parts by weight or more, 50 parts by weight or more, 100 parts by weight or more, 200 parts by weight or more, 300 parts by weight or more, 500 parts by weight or more, or 1,000 parts by weight or more, and 3,000 parts by weight or less, 2,000 parts by weight or less, 1,000 parts by weight or less, 500 parts by weight or less, 200 parts by weight or less, 175 parts by weight or less, 150 parts by weight or less, 125 parts by weight or less, 100 parts by weight or less, 80 parts by weight or less, 60 parts by weight or less, 40 parts by weight or less, 20 parts by weight or less, or 10 parts by weight or less based on 1 part by weight of the wax.

The amount of the organic solvent may be 1 part by weight or more, 3 parts by weight or more, 5 parts by weight or more, 10 parts by weight or more, 20 parts by weight or more, 30 parts by weight or more, 40 parts by weight or more, 50 parts by weight or more, 100 parts by weight or more, 200 parts by weight or more, 300 parts by weight or more, 500 parts by weight or more, or 1,000 parts by weight or more, and 3,000 parts by weight or less, 2,000 parts by weight or less, 1,000 parts by weight or less, 500 parts by weight or less, 200 parts by weight or less, 175 parts by weight or less, 150 parts by weight or less, 125 parts by weight or less, 100 parts by weight or less, 80 parts by weight or less, 60 parts by weight or less, 40 parts by weight or less, 20 parts by weight or less, or 10 parts by weight or less relative to 1 part by weight of the wax.

### {Silicone}

The repellent in the present disclosure may include silicone (polyorganosiloxane). Containing the silicone enables providing favorable texture and durability in addition to favorable liquid-repellency.

As the silicone, a known silicone can be used, and examples of the silicone include a polydimethylsiloxane and modified silicones (for example, amino-modified silicone, epoxy-modified silicone, carboxy-modified silicone, and methylhydrogen silicone). For example, the silicone may be silicone wax having waxy properties. These may be used singly or in combination of two or more thereof.

A weight average molecular weight of the silicone may be 1,000 or more, 10,000 or more, or 50,000 or more, and may be 500,000 or less, 2,500,000 or less, 100,000 or less, or 50,000 or less.

### [Amount of Silicone]

The amount of silicone is 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less.

### {Organic Acid}

The repellent of the present disclosure may contain an organic acid. As the organic acid, a known organic acid can be used. Examples of the organic acid preferably include, for example, a carboxylic acid, a sulfonic acid, and a sulfinic acid, with the carboxylic acid being particularly preferred. Examples of the carboxylic acid include, for example, formic acid, acetic acid, propionic acid, butyric acid, oxalic acid, succinic acid, glutaric acid, adipic acid, malic acid, and citric acid, with the formic acid or acetic acid being particularly preferred. In the present disclosure, one type of organic acid may be used, or two or more thereof may be combined for use. For example, formic acid and acetic acid may be combined for use.

### [Amount of Organic Acid]

The amount of organic acid may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less. The amount of organic acid may be adjusted so that a pH of the repellent is 3 to 10, for example 5 to 9, particularly 6 to 8. For example, the repellent may be acidic (pH of 7 or less, for example 6 or less).

### {Inorganic acid}

The repellent according to the present disclosure may comprise an inorganic acid. The inorganic acid may be a known inorganic acid. Examples of inorganic acids include hydrogen chloride, hydrogen bromide, hydrogen iodide, nitric acid, boric acid, sulfuric acid and phosphoric acid. In the present disclosure, one inorganic acid may be used, or two or more of them may be used in combination. The addition of inorganic acid can improve the stability of the aqueous dispersion.

### [Amount of inorganic acid]

The amount of inorganic acid may be 0.1 part by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, and 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less based on 100 parts by weight of the wax. The amount of the inorganic acid may be adjusted so that the repellent has a pH of 3 to 10, for example, 5 to 9, and in particular, 6 to 8. The repellent may be acidic (may have a pH of 7 or less, for example, 6 or less).

### {Curing Agent}

The repellent of the present disclosure may contain a curing agent (active hydrogen-reactive compound or active hydrogen-containing compound).

The curing agent (cross-linking agent) in the repellent can effectively cure the repellent. The curing agent may be an active hydrogen-reactive compound or an active hydrogen-containing compound, which reacts with an active hydrogen or an active hydrogen-reactive group. Examples of the active hydrogen-reactive compound include an isocyanate compound, epoxy compound, chloromethyl group-containing compound, carboxyl group-containing compound, and hydrazide compound. Examples of the active hydrogen-containing compound include a hydroxyl group-containing compound, an amino group-containing compound and a carboxyl group-containing compound, a ketone group-containing compound, a hydrazide compound, and a melamine compound.

The curing agent may contain an isocyanate compound. The isocyanate compound may be a polyisocyanate compound. The polyisocyanate compound is a compound having two or more isocyanate groups in one molecule. The polyisocyanate compound serves as a cross-linking agent. Examples of the polyisocyanate compound include, for example, an aliphatic polyisocyanate, an alicyclic polyisocyanate, an araliphatic polyisocyanate, an aromatic polyisocyanate, and derivatives of these polyisocyanates. The isocyanate compound may be a blocked isocyanate compound (for example, a blocked polyisocyanate compound). The blocked isocyanate compound is a compound in which an isocyanate group of an isocyanate compound is masked with a blocking agent to inhibit reaction.

Examples of the aliphatic polyisocyanates are aliphatic triisocyanates such as trimethylene diisocyanate, tetramethylene diisocyanate, hexamethylene diisocyanate, pentamethylene diisocyanate, 1,2-propylene diisocyanate, 1,2-butylene diisocyanate, 2,3-butylene diisocyanate, 1,3-butylene diisocyanate, 2,4,4- or 2,2,4-trimethylhexamethylene diisocyanate, an aliphatic diisocyanate of 2,6-diisocyanatomethylcaproate, and aliphatic triisocyanates such as lysine ester triisocyanate, 1,4,8-triisocyanateoctane, 1,6,11-triisocyanatoundecane, 1,8-diisocyanato-4-isocyanatomethyloctane, 1,3,6-triisocyanatohexane, 2,5,7-trimethyl-1,8-diisocyanato-5-isocyanatomethyloctane. These may be used singly or in combination of two or more thereof.

Examples of the alicyclic polyisocyanates include, for example, an alicyclic diisocyanate and an alicyclic triisocyanate. Specific examples of the alicyclic polyisocyanate include 1,3-cyclopentene diisocyanate, 3-isocyanatomethyl-3,5,5-trimethylcyclohexyl isocyanate (isophorone diisocyanate), and 1,3,5-triisocyanatocyclohexane. These may be used singly or in combination of two or more thereof.

Examples of the aromatic-aliphatic polyisocyanate include an aromatic-aliphatic diisocyanate and aromatic-aliphatic triisocyanate. Specific examples of the araliphatic polyisocyanate include 1,3- or 1,4-xylylene diisocyanate or a mixture thereof, 1,3- or 1,4-bis(1-isocyanato-1-methylethyl)benzene (tetramethyl xylylene diisocyanate) or a mixture thereof, and 1,3,5-triisocyanatomethylbenzene. These may be used singly or in combination of two or more thereof.

Examples of the aromatic polyisocyanates include an aromatic diisocyanate, aromatic triisocyanate, and aromatic tetraisocyanate. Specific examples of the aromatic polyisocyanate include, for example, m-phenylene diisocyanate, p-phenylene diisocyanate, 4,4'-diphenyl diisocyanate, 1,5-naphthalene diisocyanate, 2,4'- or 4,4'-diphenylmethane diisocyanate, or a mixture thereof, 2,4- or 2,6-tolylene diisocyanate or a mixture thereof, triphenylmethane-4,4',4"-triisocyanate, and 4,4'-diphenylmethane-2,2',5,5'-tetraisocyanate. These may be used singly or in combination of two or more thereof.

Examples of the derivative of the polyisocyanate include various derivatives such as a dimer, trimer, biuret, allophanate, carbodiimide, urethodione, urethoimine, isocyanurate, and iminooxadiazinedione of the aforementioned polyisocyanate compounds. These may be used singly or in combination of two or more thereof.

These polyisocyanates can be used singly or in combination of two or more thereof.

As the polyisocyanate compound, a blocked polyisocyanate compound (blocked isocyanate), which is a compound obtained by blocking isocyanate groups of the polyisocyanate compound with a blocking agent, is preferably used. The blocked polyisocyanate compound is preferably used because it is relatively stable even in solution and can be used in the same solution as solution of the repellent.

The blocking agent is an agent that blocks free isocyanate groups. The blocked polyisocyanate compound, for example, can be heated 100°C or higher, for example, 130°C or higher to regenerate isocyanate groups, facilitating a reaction with hydroxyl groups. Examples of the blocking agent include, for example, a phenolic compound, lactam-based compound, aliphatic alcohol-based compound, and oxime-based compound. The polyisocyanate compound may be used singly or in combination of two or more thereof.

The epoxy compound is a compound having an epoxy group. Examples of the epoxy compound include epoxy compounds having a polyoxyalkylene group, such as a polyglycerol polyglycidyl ether and a polypropylene glycol diglycidyl ether; as well as a sorbitol polyglycidyl ether.

The chloromethyl group-containing compound is a compound having a chloromethyl group. Examples of the chloromethyl group-containing compound include, for example, a chloromethyl polystyrene.

The carboxyl group-containing compound is a compound having a carboxyl group. Examples of the carboxyl group-containing compound include, for example, a (poly)acrylic acid, and a (poly)methacrylic acid.

Specific examples of the ketone group-containing compound include, for example, a (poly)diacetone acrylamide, and diacetone alcohol.

Specific examples of the hydrazide compound include, for example, hydrazine, a carbohydrazide, and adipic acid hydrazide.

Specific examples of the melamine compound include, for example, a melamine resin and a methyl etherified melamine resin.

### [Amount of Curing Agent]

The amount of the curing agent may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, and 5 parts by weight or less.

### {Other Component}

The repellent may contain a component other than the aforementioned components. Examples of the other components include, for example, polysaccharides, a paper strengthening agent, an agglomerating agent, a yield improver, a coagulant, a binder resin, an anti-slip agent, a sizing agent, a paper strengthening agent, a filler, an antistatic agent, an antiseptic agent, an ultraviolet absorber, an antibacterial agent, a deodorant, and a fragrance. These may be used singly or in combination of two or more thereof. In addition to the above components, as other components, for example, other water-repellent and/or oil-repellent agents, a dispersant, a texture modifier, a softening agent, a flame retarder, a coating material fixing agent, a wrinkle-resistant agent, a drying rate adjuster, a cross-linking agent, a film formation agent, a compatibilizer, an antifreezing agent, a viscosity adjuster, an ultraviolet absorber, an antioxidant, a pH adjuster, an insect repellent, an antifoaming agent, an anti-shrinkage agent, a laundry wrinkle-resistant agent, a shape retention agent, a drape retention agent, an ironing improving agent, a brightening agent, a whitening agent, fabric softening clay, a migration-proofing agent such as a polyvinylpyrrolidone, a polymer dispersant, a soil release agent, a scum dispersant, a fluorescent brightening agent such as 4,4-bis(2-sulfostyryl)biphenyldisodium (Tinopal CBS-X manufactured by Ciba Specialty Chemicals Plc), a dye fixing agent, an anti-color fading agent such as 1,4-bis(3-aminopropyl) piperazine, a stain removing agent, enzymes such as cellulase, amylase, protease, lipase, and keratinase as fiber surface modifiers, a foam inhibitor, and silk protein powder that can impart texture and functions of silk such as moisture absorption and release properties, and surface modified products or emulsified dispersions thereof (for example, K-50, K-30, K-10, A-705, S-702, L-710, FP series (Idemitsu Petrochemical Co., Ltd.), hydrolyzed silk liquid (Jomo), SILKGEN G Soluble S (ICHIMARU PHARCOS Co., Ltd.)), an antifouling agent (for example, a nonionic polymer compound composed of an alkylene terephthalate and/or an alkylene isophthalate units and a polyoxyalkylene unit (for example, FR627 manufactured by GOO CHEMICAL CO., LTD.), SRC-1 manufactured by Clariant (Japan), K. K.), can be compounded. These may be used singly or in combination of two or more thereof.

### [Amount of Other Component]

Each amount or the total amount of other components may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less.

### <Pulp composition>

The pulp composition of the present disclosure comprises pulp and a repellent component. The pulp composition of the present disclosure is obtained by treating pulp with a repellent.

### {Pulp}

The pulp composition includes pulp, and the pulp, which is a pulp substrate, is treated with a repellent. The pulp substrate may be in the form of pulp alone, pulp slurry, or a pulp product. Examples of pulp substrates include bleached or unbleached chemical pulp such as kraft pulp or sulfite pulp; bleached or unbleached high-yield pulp such as groundwood pulp, mechanical pulp, or thermomechanical pulp; pulp slurry including the above pulp; and a pulp product such as paper, a paper container and a paper formed article made of wastepaper pulp such as wastepaper of newspapers, magazines and cardboard, or deinked wastepaper. Specific examples of the pulp products include, for example, a food packaging material, a food container, gypsum liner board base paper, coated base paper, medium-quality paper, a general liner and core, neutral pure white roll paper, a neutral liner, a rust-proof liner, and metal pasted paper, kraft paper, neutral printing writing paper, neutral coated base paper, neutral PPC paper, neutral thermal paper, neutral pressure-sensitive base paper, neutral inkjet paper and neutral information paper, and molded paper (mold container). Preferred examples of pulp products include a food packaging material and a food container, and in particular, a pulp formed article for food contact.

The amount of pulp may be 0.1% by weight or more, 0.5% by weight or more, 1% by weight or more, 3% by weight or more, 5% by weight or more, 10% by weight or more, 20% by weight or more, 30% by weight or more, 50% by weight or more, 75% by weight or more, or 90% by weight or more, and 99% by weight or less, 75% by weight or less, 50% by weight or less, 40% by weight or less, 30% by weight or less, 20% by weight or less, 10% by weight or less, 5% by weight or less, 4% by weight or less, or 3% by weight or less in the pulp composition. Typically, when the pulp composition is prepared by internal addition, the amount of pulp may be 30% by weight or less in the pulp composition; when the pulp composition is prepared by external addition, the amount of pulp may be 75% by weight or more in the pulp composition.

### {Liquid medium}

The pulp composition may comprise a liquid medium. The liquid medium may be water, an organic solvent, or a mixture of water and an organic solvent. The liquid medium is typically an aqueous medium, and in particular, water. The liquid medium may comprise a liquid medium derived from repellent.

### [Amount of liquid medium]

The amount of the liquid medium may be 0.1% by weight or more, 0.5% by weight or more, 1% by weight or more, 3% by weight or more, 5% by weight or more, 10% by weight or more, 20% by weight or more, 30% by weight or more, 50% by weight or more, 75% by weight or more, 90% by weight or more, or 95% by weight or more, and 99% by weight or less, 75% by weight or less, 50% by weight or less, 40% by weight or less, 30% by weight or less, 20% by weight or less, 10% by weight or less, 5% by weight or less, 4% by weight or less, or 3% by weight or less in the pulp composition. Typically, when the pulp composition is prepared by internal addition, the amount of the liquid medium is 50% by weight or more, and in particular 90% by weight or more in the pulp composition; when the pulp composition is prepared by external addition, the amount of the liquid medium is 30% by weight or less, and in particular, 10% by weight or less in the pulp composition.

### {Repellent}

The pulp composition may comprise wax included in the repellent. The repellent will be separately described in <Repellent>.

### [Amount of repellent]

The amount of the repellent added to the pulp (also referred to as a pulp substrate) may be adjusted to achieve the desired amount of wax. The amount of the wax may be 0.1% by weight or more, 0.3% by weight or more, 0.5% by weight or more, 0.75% by weight or more, 1.0% by weight or more, 2.0% by weight or more, or 3.0% by weight or more, and 10% by weight or less, 7.5% by weight or less, 5.0% by weight or less, 4.0% by weight or less, 3.0% by weight or less, 2.0% by weight or less, 1.0% by weight or less, 0.75% by weight or less, or 0.5% by weight or less, preferably 5.0% by weight or less, and more preferably 3.0% by weight or less based on the pulp.

In the external addition treatment, the amount of the wax contained in the coating layer may be 0.01 g/m² or more, 0.03 g/m² or more, 0.05 g/m² or more, 0.1 g/m² or more, 0.3 g/m² or more, 0.5 g/m² or more, or 1.0 g/m² or more, and 5.0 g/m² or less, 4.0 g/m² or less, 3.0 g/m² or less, 2.0 g/m² or less, 1.0 g/m² or less, 0.5 g/m² or less, 0.3 g/m² or less, or 0.1 g/m² or less.

### {Paper strength agent}

The pulp composition may comprise a paper strength agent. Examples of paper strength agents include:
a polyacrylamide paper strength agent such as cationic polyacrylamide, anionic polyacrylamide and amphoteric polyacrylamide;
a polysaccharide paper strength agent such as starch, enzyme modified starch, thermochemically modified starch, oxidized starch, esterified starch, etherified starch (e.g., hydroxyethylated starch), aldehyde starch, cationized starch, starch, xanthan gum, gum karaya, welan gum, guar gum, pectin, tamarind gum, carrageenan, chitosan, gum arabic, locust bean gum, cellulose, alginic acid, agar, dextran, cellulose, carboxymethylcellulose, hydroxyethylcellulose, hydroxypropylcellulose, chitin nanofiber, cellulose nanofiber and pullulan, and a modified polysaccharide thereof (e.g., a modified polysaccharide into which a hydroxyl group or a cationic group is introduced);
a polyamide paper strength agent such as polyamide resin, polyamine resin, polyamide-polyamine resin, polyamide-epichlorohydrin resin, polyamide-polyamine-epichlorohydrin resin, polyamide-polyurea-formaldehyde resin and epoxidized polyamide resin;
a urea/melamine paper strength agent such as urea resin, melamine resin, urea-formaldehyde resin and melamine-formaldehyde resin;
a polyvinyl alcohol paper strength agent such as polyvinyl alcohol, completely saponified polyvinyl alcohol, partially saponified polyvinyl alcohol, carboxyl modified polyvinyl alcohol, silanol modified polyvinyl alcohol, cation modified polyvinyl alcohol and terminal alkyl modified polyvinyl alcohol; and
a styrene butadiene copolymer, polyvinyl acetate, a vinyl chloride-vinyl acetate copolymer, polyvinyl chloride, polyvinylidene chloride, polyacrylic ester, fatty acid diamide, polyethyleneimine resin and ketone aldehyde resin. A polyacrylamide paper strength agent, a polysaccharide paper strength agent and a polyamide paper strength agent are preferred as the paper strength agent in the present disclosure.

### [Amount of paper strength agent]

The total amount of the paper strength agents may be 0.1% by weight or more, 0.3% by weight or more, 0.5% by weight or more, 0.75% by weight or more, 1.0% by weight or more, 2.0% by weight or more, or 3.0% by weight or more, and 10% by weight or less, 7.5% by weight or less, 5.0% by weight or less, 4.0% by weight or less, 3.0% by weight or less, 2.0% by weight or less, 1.0% by weight or less, 0.75% by weight or less, or 0.5% by weight or less, and preferably 5.0% by weight or less based on the pulp.

The amount of the polyacrylamide paper strength agent may be 0.1% by weight or more, 0.2% by weight or more, 0.4% by weight or more, 0.6% by weight or more, 0.8% by weight or more, or 1.0, preferably 0.3% by weight or more, and 1.1% by weight or less, 0.9% by weight or less, 0.7% by weight or less, 0.5% by weight or less, or 0.3% by weight or less based on the pulp.

The amount of the polysaccharide paper strength agent may be 0.6% by weight or more, 1.0% by weight or more, 1.5% by weight or more, 2.0% by weight or more, 2.5% by weight or more, 3.0% by weight or more, 3.5% by weight or more, 4.0% by weight or more, or 4.5% by weight or more, preferably 2.0% by weight or more, and 5% by weight or less, 4.7% by weight or less, 4.2% by weight or less, 3.7% by weight or less, 3.2% by weight or less, 2.7% by weight or less, 2.2% by weight or less, or 1.7% by weight or less based on the pulp.

The amount of the polyamide paper strength agent may be 0.3% by weight or more, 0.4% by weight or more, 0.5% by weight or more, 0.6% by weight or more, 0.7% by weight or more, or 0.8% by weight or more, and 0.9% by weight or less, 0.8% by weight or less, 0.7% by weight or less, 0.6% by weight or less, 0.5% by weight or less, or 0.4% by weight or less based on the pulp.

### {Sizing agent}

The pulp composition may comprise a sizing agent. Examples of sizing agents include a cationic sizing agent, an anionic sizing agent, a neutral sizing agent and an amphoteric sizing agent, a rosin-based sizing agent (for example, an acidic rosin-based sizing agent and a neutral rosin-based sizing agent), alkyl ketene dimer and alkenyl succinic anhydride.

### [Amount of sizing agent]

The amount of the sizing agent may be 0.1% by weight or more, 0.2% by weight or more, 0.3% by weight or more, 0.5% by weight or more, 0.75% by weight or more, 1.0% by weight or more, 2.0% by weight or more, or 3.0% by weight or more, and 10% by weight or less, 7.5% by weight or less, 5.0% by weight or less, 4.0% by weight or less, 3.0% by weight or less, 2.0% by weight or less, 1.0% by weight or less, 0.75% by weight or less, or 0.5% by weight or less based on the pulp.

### {Other additives}

The pulp composition may also include an additive used for producing a pulp product in addition to the above components, such as a fixing agent (e.g., aluminum sulfate), an organic acid (e.g., formic acid, acetic acid), an agglomerating agent, a yield improver, a dye, a fluorescent dye, a slime control agent, and an antifoaming agent. While the pulp composition includes a component derived from a repellent, the components contained in the repellent which are described above may be added to the pulp composition as an additive. The pulp composition may not include a coloring agent (e.g., a dye).

The amount of the above additives may be, respectively, 0.1% by weight or more, 1% by weight or more, 3% by weight or more, 5% by weight or more, and 30% by weight or less, 20% by weight or less, 10% by weight or less, or 5% by weight or less based on the pulp.

### <Method for producing pulp product>

The method for producing a pulp product of present disclosure may comprise a step of treating a pulp substrate with a repellent (a wax addition step). The pulp substrate is treated with a repellent to give a pulp composition. The pulp composition may also be produced by the wax addition step of adding wax to pulp and a paper strength agent addition step of adding a paper strength agent to the pulp. The wax addition step and the paper strength agent addition step may be performed separately or simultaneously. A pulp product may be obtained by subjecting the resulting pulp composition to processing such as drying, heating and forming according to need.

The pulp substrate and the type and the composition of the repellent are as described in the above [Pulp composition]. The repellent of the present disclosure can be applied to a substrate as a treatment agent (particularly a surface-treating agent) by a conventionally known method. The treatment method may be a method for dispersing the repellent in the present disclosure in an organic solvent or water, if necessary, to dilute it and allowing it to adhere to an inside of a pulp substrate and/or on a surface thereof by a known method such as dip coating, spray coating, and foam coating. After drying, a pulp product to which a solid component of the repellent has been adhered, is obtained. If necessary, the repellent of the present disclosure may be applied in combination of a suitable cross-linking agent, and curing may be carried out. A concentration of the repellent in a treatment agent brought into contact with a pulp substrate may be appropriately changed depending on its use, and may be 0.01 to 10% by weight, for example 0.05 to 5% by weight.

The repellent can be applied to a pulp substrate by any of methods known for treating a pulp substrate with liquid. The pulp substrate may be immersed in the repellent or mixed with the repellent, or solution may be adhered or sprayed onto the substrate. The treated pulp substrate is preferably dried and cured by heating in order to develop liquid-repellency. The heating temperature may be, for example, 100°C to 200°C, 100°C to 170°C, or 100°C to 120°C. In the present disclosure, the heating time may be 5 seconds to 60 minutes, for example, 30 seconds to 3 minutes.

The method of treatment of the pulp substrate may be an internal addition treatment method in which a repellent is added to pulp before papermaking (e.g., pulp slurry), or an external addition treatment method in which a repellent is applied to paper after papermaking (e.g., a pulp product). Examples of internal addition treatment include mixing and dipping, and the internal addition treatment may include a step of adding a repellent to a pulp slurry and mixing with stirring. Examples of external addition treatment include spraying and coating, and more specifically a pound-type two-roll size press, a gate roll type, and a rod metering type size press. The treatment may be external addition treatment or internal addition treatment. For example, when the pulp substrate is paper, the repellent may be applied to paper, or solution may be adhered or sprayed onto paper, or the repellent may be mixed with pulp slurry before papermaking to perform treatment.

The method of treatment may be internal addition treatment in which a repellent is added to pulp slurry before papermaking. The internal addition treatment method may include, but is not limited to, one or more of a step of adding the repellent to pulp slurry and stirring and mixing them; a step of sucking and dehydrating the pulp composition prepared in the step through a net-like body of predetermined shape and depositing the pulp composition then to form a pulp formed article intermediate; and a step of molding and drying the pulp formed article intermediate by using a heated forming mold to obtain a pulp formed article. After having been lightly dried at room temperature or elevated temperature, the treated paper may be arbitrarily subjected to heat treatment, depending on the nature of the paper. Temperature of the heat treatment may be 150°C or higher, 180°C or higher, or 210°C or higher, and may be 300°C or lower, 250°C or lower, or 200°C or lower, particularly 80°C to 180°C. Carrying out the heat treatment in such a temperature range enables exhibiting, for example, excellent oil resistance and water resistance. The pulp substrate which has undergone internal addition treatment may be subjected to external addition treatment to be treated with the repellent, allowing a further wax and a further paper strength agent to be adhered to the surface. Examples of further waxes and further paper strength agents are as described above, but not limited thereto.

The treatment method may be an external addition treatment in which the repellent is applied to pulp substrate after papermaking. A size press used in an external addition treatment, can be divided into the following types depending on a coating method. One coating method involves supplying a coating liquid (size liquid) to a nip portion formed by passing paper between two rubber rolls, creating a pool of the coating liquid called a pond, and allowing the paper to pass through this pool to coat both sides of the paper with the size liquid, which is a method employed for a so-called pound-type two-roll size press. Another coating method is a method used for a gate roll type size press in which a size liquid is applied by a surface transfer type, and a rod metering type size press. In the pound-type two-roll size press, the size liquid easily penetrates into an inside of paper, and in the surface transfer type, a size liquid component is likely to stay on a surface of the paper. In the surface transfer type, a coating layer is likely to stay on a surface of paper more than in the pound-type two-roll size press, and the amount of coating layer formed on the surface is more than in the pound-type two-roll size press. In the present disclosure, even in the case of using the former pound-type two-roll size press, performance can be imparted to paper. After having been lightly dried at room temperature or elevated temperature, the paper treated in such a manner is arbitrarily accompanied by heat treatment that can have a temperature range of up to 300°C, for example up to 200°C, and particularly the temperature range of 80°C to 180°C, depending on the nature of the paper, as a result of which excellent oil resistance, water resistance, and the like can be exhibited.

### <Strength of pulp molded article>

### {Dry strength}

The dry strength of the pulp molded article of the present disclosure is not limited, and is evaluated based on the specific tensile strength in the dry condition which is measured according to JIS P 8113:2006. The specific dry tensile strength is obtained by dividing dry tensile strength by density.

The pulp molded article of the present invention has a dry strength (specific dry tensile strength) of preferably 20.0 Nm/g or more, 25.0 Nm/g or more, 30.0 Nm/g or more, more preferably 35.0 Nm/g or more, and further preferably 40.0 Nm/g or more. The upper limit is not limited, and is 200 Nm/g or less, more preferably 100 Nm/g or less, and further preferably 50 Nm/g or less from the viewpoint of ease of manufacture.

Adding wax to the pulp substrate reduces the dry strength of the resulting pulp product. Although the method of addition is not limited, reduction in dry strength is larger in internal addition treatment in which wax is added to pulp slurry before papermaking, than that in external addition treatment in which wax is applied to paper after papermaking. In the present disclosure, reduction in dry strength has been found to be prevented by employing a specific composition even when wax is used.

### {Wet strength}

The wet strength of the pulp molded article of the present disclosure is not limited, and is evaluated based on the specific wet tensile strength in the wet condition which is measured according to JIS P 8135:0998. The specific wet tensile strength is obtained by dividing wet tensile strength by density.

The pulp molded article of the present invention has a wet strength (specific wet tensile strength) of preferably 3.0 Nm/g or more, 6.0 Nm/g or more, 8.0 Nm/g or more, 10.0 Nm/g or more, 12.0 Nm/g or more, or 14.0 Nm/g or more, preferably 3.0 Nm/g or more, more preferably 4.0 Nm/g or more, and further preferably 5.0 Nm/g or more, and even more preferably 8.0 Nm/g or more. The upper limit is not limited, and may be 20 Nm/g or less, 18 Nm/g or less, 16 Nm/g or less, or 15 Nm/g or less, preferably 16 Nm/g or less, and for example, 14 Nm/g or less from the viewpoint of ease of manufacture.

Adding wax to the pulp substrate reduces the wet strength of the resulting pulp product. Although the method of addition is not limited, reduction in wet strength is larger in internal addition treatment in which an oil resistant agent is added to pulp slurry before papermaking, than that in external addition treatment in which an oil resistant agent is applied to paper after papermaking. In the present disclosure, reduction in wet strength has been found to be prevented by employing a specific composition even when wax is used.

### Examples

Hereinafter, the present disclosure will be described in detail with reference to Examples, but the present disclosure is not limited to these Examples.

### <Test Method>

The test procedures are as follows.

### [Dry tensile strength]

Tensile strength was measured by the method according to JIS P 8113.

### [Wet tensile strength]

Wet strength was measured by the method according to JIS P 8135.

### [Oil resistance]

After pouring 100 ml of corn oil at 50°C into the pulp molded article and allowing it to stand at room temperature for 30 minutes, the corn oil was removed from the pulp molded article, and the degree of staining in the pulp molded article was evaluated. The evaluation scores were set as follows according to the degree of staining.
5: No stains inside the pulp mold.
4: Stains inside the pulp mold. No stains on the backside.
3: Stains the inside the pulp mold. Slight stain bleed out on the backside.
2: Stains inside the pulp mold. The area of stain bleed out to the backside is less than 50% of the total area.
1: Stains inside the pulp mold. The area of stain bleed out to the backside is 50% or more and less than 100% of the total area.
0: Stains over the backside.

### [Moldability]

Whether poor dehydration and poor adhesion occurred in molding of the pulp molded article or not was assessed based on the following criteria.
∘: without poor dehydration and poor molding
x: with poor dehydration and poor molding occurred

### [Re-disintegrating properties]

10 g of the respective molded pulp molded articles was crushed into 3 to 4 cm square pieces and dipped in tap water at 20°C. The pulp molded article was diluted to a concentration of 1.5%, and then was disintegrated using a disintegrator at a rotation speed of 3,000 rpm for 20 minutes. The degree of disintegration of the paper pieces of the pulp slurry obtained was evaluated according to the following criteria.
∘: Paper pieces completely disintegrated into fibers
x: Paper pieces remaining without being disintegrated

### [Example 1]

2,000 g of a 0.5% by weight aqueous dispersion of a mixture of 70 parts of broad leaf tree bleached kraft pulp and 30 parts of needle bleached kraft pulp beaten to a freeness (Canadian Standard Freeness) of 500 cc, was added with stirring. Then a wax emulsion (repellent) including 2 g of paraffin wax, 0.05 g of benzalkonium chloride, 0.04 g of abietic acid (rosin sizing agent), 0.04 g of formic acid, 0.04 g of acetic acid and 7.83 g of water was added thereto at a ratio of 1.85% in terms of the amount of wax based on the pulp, and stirring was continued for 1 minute; next, a polyacrylamide paper strength agent (product name: T-FC109 made by Seiko PMC Corporation) was added thereto at a ratio of 0.1% based on the pulp and stirring was continued for 1 minute; then aluminum sulfate was added thereto at a ratio of 0.04% in terms of aluminum oxide based on the pulp and stirring was continued for 1 minute; and an alkyl ketene dimer (AKD) (Hercon (registered trademark) made by Solenis) was added thereto at a ratio of 0.45% based on the pulp and stirring was continued for 1 minute.

The pulp composition obtained above was placed in a metal tank. A metal forming mold with many suction holes was installed at the lower part of the tank, and a net-like body was arranged thereon. From the opposite side of the forming mold to the side where the net-like body was arranged, the pulp composition was suctioned and dehydrated through the forming mold and the net-like body by a vacuum pump, and solids (pulp, etc.) contained in the pulp composition were allowed to deposit on the net-like body to obtain a pulp molded article intermediate. The resulting pulp molded article intermediate was then dried by applying pressure thereto from the tops and bottoms of male and female forming molds made of metal, which have been heated to 60 to 200°C. Thus, a pulp molded article having a basis weight of 500 gsm formed into the shape of a container was produced. The content ratio of the respective components in the resulting pulp molded article based on the pulp, and the results of evaluation of the specific tensile strength, oil resistance, moldability and re-disintegrating properties are shown in Table 1. For the specific tensile strength, at least one of the dry tensile strength and the wet tensile strength was evaluated (the same below).

### [Example 2]

The experiment was performed in the same manner as in Example 1 except for adding the polyacrylamide paper strength agent at a ratio of 0.5% based on the pulp. The content ratio of the respective components in the resulting pulp molded article based on the pulp, and the results of evaluation of the specific tensile strength, oil resistance, moldability and re-disintegrating properties are shown in Table 1.

### [Example 3]

The experiment was performed in the same manner as in Example 1 except for adding the polyacrylamide paper strength agent at a ratio of 1.1% based on the pulp. The content ratio of the respective components in the resulting pulp molded article based on the pulp, and the results of evaluation of the specific tensile strength, oil resistance, moldability and re-disintegrating properties are shown in Table 1.

### [Example 4]

The experiment was performed in the same manner as in Example 2 except for adding wax emulsion at a ratio of 0.20% in terms of the amount of wax. The content ratio of the respective components in the resulting pulp molded article based on the pulp, and the results of evaluation of the specific tensile strength, oil resistance, moldability and re-disintegrating properties are shown in Table 1.

### [Example 5]

The experiment was performed in the same manner as in Example 2 except for adding wax emulsion at a ratio of 10.0% in terms of the amount of wax. The content ratio of the respective components in the resulting pulp molded article based on the pulp, and the results of evaluation of the specific tensile strength, oil resistance, moldability and re-disintegrating properties are shown in Table 1.

### [Example 6]

The experiment was performed in the same manner as in Example 1 except for adding a polysaccharide paper strength agent (product name CATOSIZE380H made by Ingredion) instead of the polyacrylamide paper strength agent at a ratio of 0.6% based on the pulp. The content ratio of the respective components in the resulting pulp molded article based on the pulp, and the results of evaluation of the specific tensile strength, oil resistance, moldability and re-disintegrating properties are shown in Table 1.

### [Example 7]

The experiment was performed in the same manner as in Example 6 except for adding the polysaccharide paper strength agent at a ratio of 1.5% based on the pulp. The content ratio of the respective components in the resulting pulp molded article based on the pulp, and the results of evaluation of the specific tensile strength, oil resistance, moldability and re-disintegrating properties are shown in Table 1.

### [Example 8]

The experiment was performed in the same manner as in Example 6 except for adding the polysaccharide paper strength agent at a ratio of 5.0% based on the pulp. The content ratio of the respective components in the resulting pulp molded article based on the pulp, and the results of evaluation of the specific tensile strength, oil resistance, moldability and re-disintegrating properties are shown in Table 1.

### [Example 9]

The experiment was performed in the same manner as in Example 1 except for adding a polyamide paper strength agent (product name: WS4020 made by Seiko PMC Corporation) instead of the polyacrylamide paper strength agent at a ratio of 0.3% based on the pulp. The content ratio of the respective components in the resulting pulp molded article based on the pulp, and the results of evaluation of the specific tensile strength, oil resistance, moldability and re-disintegrating properties are shown in Table 2.

### [Example 10]

The experiment was performed in the same manner as in Example 9 except for adding the polyamide paper strength agent at a ratio of 0.6% based on the pulp. The content ratio of the respective components in the resulting pulp molded article based on the pulp, and the results of evaluation of the specific tensile strength, oil resistance, moldability and re-disintegrating properties are shown in Table 2.

### [Example 11]

The experiment was performed in the same manner as in Example 9 except for adding the polyamide paper strength agent at a ratio of 0.9% based on the pulp. The content ratio of the respective components in the resulting pulp molded article based on the pulp, and the results of evaluation of the specific tensile strength, oil resistance, moldability and re-disintegrating properties are shown in Table 2.

### [Comparative Example 1]

The experiment was performed in the same manner as in Example 1 except for not adding the wax emulsion or the polyacrylamide paper strength agent. The content ratio of the respective components in the resulting pulp molded article based on the pulp, and the results of evaluation of the specific tensile strength, oil resistance, moldability and re-disintegrating properties are shown in Table 1.

### [Comparative Example 2]

The experiment was performed in the same manner as in Example 1 except for not adding the polyacrylamide paper strength agent. The content ratio of the respective components in the resulting pulp molded article based on the pulp, and the results of evaluation of the specific tensile strength, oil resistance, moldability and re-disintegrating properties are shown in Table 1.

### [Comparative Example 3]

The experiment was performed in the same manner as in Example 1 except for adding the polyacrylamide paper strength agent at a ratio of 0.02% based on the pulp. The content ratio of the respective components in the resulting pulp molded article based on the pulp, and the results of evaluation of the specific tensile strength, oil resistance, moldability and re-disintegrating properties are shown in Table 1.

### [Comparative Example 4]

The experiment was performed in the same manner as in Example 1 except for adding the polyacrylamide paper strength agent at a ratio of 1.85% based on the pulp. The content ratio of the respective components in the resulting pulp molded article based on the pulp, and the results of evaluation of the specific tensile strength, oil resistance, moldability and re-disintegrating properties are shown in Table 1.

### [Comparative Example 5]

The experiment was performed in the same manner as in Comparative Example 2 except for adding wax emulsion at a ratio of 0.20% in terms of the amount of wax. The content ratio of the respective components in the resulting pulp molded article based on the pulp, and the results of evaluation of the specific tensile strength, oil resistance, moldability and re-disintegrating properties are shown in Table 1.

### [Comparative Example 6]

The experiment was performed in the same manner as in Comparative Example 2 except for adding wax emulsion at a ratio of 10.0% in terms of the amount of wax. The content ratio of the respective components in the resulting pulp molded article based on the pulp, and the results of evaluation of the specific tensile strength, oil resistance, moldability and re-disintegrating properties are shown in Table 1.

### [Comparative Example 7]

The experiment was performed in the same manner as in Example 6 except for adding the polysaccharide paper strength agent at a ratio of 8.0% based on the pulp. The content ratio of the respective components in the resulting pulp molded article based on the pulp, and the results of evaluation of the specific tensile strength, oil resistance, moldability and re-disintegrating properties are shown in Table 1.

### [Comparative Example 8]

The experiment was performed in the same manner as in Example 6 except for externally treating, with the wax emulsion, the surface of the molded article after molding pulp instead of the internal addition. The content ratio of the respective components in the resulting pulp molded article based on the pulp, and the results of evaluation of the specific tensile strength, oil resistance, moldability and re-disintegrating properties are shown in Table 1.

### [Comparative Example 9]

The experiment was performed in the same manner as in Example 9 except for adding the polyamide paper strength agent at a ratio of 1.2% based on the pulp. The content ratio of the respective components in the resulting pulp molded article based on the pulp, and the results of evaluation of the specific tensile strength, oil resistance, moldability and re-disintegrating properties are shown in Table 2.

**[Table 1] Specific dry tensile strength**

| | | Ex. 1 | Ex. 2 | Ex. 3 | Ex. 4 | Ex. 5 | Ex. 6 | Ex. 7 | Ex. 8 | Com. Ex. 1 | Com. Ex.2 | Com. Ex.3 | Com. Ex.4 | Com. Ex.5 | Com. Ex.6 | Com. Ex.7 | Com. Ex.8 |
|---|---|---|---|---|---|---|---|---|---|---|---|---|---|---|---|---|---|
| Polyacrylamide paper strength agent | dry% | 0.1 | 0.5 | 1.1 | 0.5 | 0.5 | 0 | 0 | 0 | 0 | 0 | 0.02 | 1.85 | 0 | 0 | 0 | 0 |
| Polysaccharide paper strength agent | dry% | 0 | 0 | 0 | 0 | 0 | 0.6 | 1.5 | 5 | 0 | 0 | 0 | 0 | 0 | 0 | 8.0 | 0 |
| Polyamide paper strength agent | dry% | 0 | 0 | 0 | 0 | 0 | 0 | 0 | 0 | 0 | 0 | 0 | 0 | 0 | 0 | 0 | 0 |
| Wax emulsion | dry% | 1.85 | 1.85 | 1.85 | 0.2 | 10.0 | 1.85 | 1.85 | 1.85 | 0 | 1.85 | 1.85 | 1.85 | 0.2 | 10.0 | 1.85 | 1.85 |
| Specific dry tensile strength | N·g/m | 23.0 | 31.3 | 39.8 | 37.3 | 26.9 | 26.0 | 30.8 | 37.6 | 26.9 | 21.3 | 21.3 | 56.1 | 26.0 | 17.9 | 39.9 | 25.1 |
| Oil resistance | Evaluation score | 4 | 4 | 4 | 4 | 4 | 4 | 4 | 4 | 0 | 4 | 4 | 4 | 4 | 4 | 4 | 4 |
| Moldability | ○or× | ○ | ○ | ○ | ○ | ○ | ○ | ○ | ○ | ○ | ○ | ○ | × | ○ | ○ | × | ○ |
| Re-disintegrating properties | ○or× | ○ | ○ | ○ | ○ | ○ | ○ | ○ | ○ | ○ | ○ | ○ | ○ | ○ | ○ | ○ | ○ |

**[Table 2] Specific wet tensile strength**

| | | Ex. 9 | Ex. 10 | Ex. 11 | Com. Ex.2 | Com. Ex.9 |
|---|---|---|---|---|---|---|
| Polyacrylamide paper strength agent | dry% | 0 | 0 | 0 | 0 | 0 |
| Polysaccharide paper strength agent | dry% | 0 | 0 | 0 | 0 | 0 |
| Polyamide paper strength agent | dry% | 0.3 | 0.6 | 0.9 | 0 | 1.2 |
| Wax emulsion | dry% | 1.85 | 1.85 | 1.85 | 1.85 | 1.85 |
| Specific wet tensile strength | N·g/m | 8.7 | 12.7 | 14.1 | 1.2 | 14.7 |
| Oil resistance | Evaluation score | 4 | 4 | 4 | 4 | 4 |
| Moldability | ○or× | ○ | ○ | ○ | ○ | ○ |
| Re-disintegrating properties | ○or× | ○ | ○ | ○ | ○ | × |

## Claims

1. A pulp composition comprising pulp, a wax and a paper strength agent, wherein
the paper strength agent is at least one selected from the group consisting of a polyacrylamide paper strength agent, a polysaccharide paper strength agent and a polyamide paper strength agent,
the amount of the wax is 0.2% by weight or more and 10.0% by weight or less based on the pulp, and
the pulp composition satisfies at least one of the following (1) to (3):
(1) an amount of the polyacrylamide paper strength agent is 0.1% by weight or more and 1.1% by weight or less based on the pulp;
(2) an amount of the polysaccharide paper strength agent is 0.6% by weight or more and 5.0% by weight or less based on the pulp; and
(3) an amount of the polyamide paper strength agent is 0.3% by weight or more and 0.9% by weight or less based on the pulp.

2. The pulp composition according to claim 1, wherein the amount of the polyacrylamide paper strength agent is 0.1% by weight or more and 1.1% by weight or less based on the pulp.

3. The pulp composition according to claim 1 or 2, wherein the amount of the polysaccharide paper strength agent is 0.6% by weight or more and 5% by weight or less based on the pulp.

4. The pulp composition according to any one of claims 1 to 3, wherein the amount of the polyamide paper strength agent is 0.3% by weight or more and 0.9% by weight or less based on the pulp.

5. The pulp composition according to any one of claims 1 to 4, wherein the wax is petroleum wax.

6. The pulp composition according to any one of claims 1 to 5, wherein the wax is at least one selected from the group consisting of paraffin wax and microcrystalline wax.

7. The pulp composition according to any one of claims 1 to 6, wherein the wax is paraffin wax.

8. The pulp composition according to any one of claims 1 to 7, comprising at least one selected from the group consisting of benzalkonium chloride, formic acid, acetic acid and rosin.

9. The pulp composition according to any one of claims 1 to 8, which is free of dye.

10. The pulp composition according to any one of claims 1 to 9, wherein
the wax is paraffin wax, and
the pulp composition comprises at least one selected from the group consisting of benzalkonium chloride, formic acid, acetic acid and rosin.

11. A pulp formed article formed of the pulp composition according to any one of claims 1 to 10.

12. The pulp formed article according to claim 11, comprising a further wax and a further paper strength agent adhering to the surface.

13. The pulp formed article according to claim 11 or 12, which is for food contact.

14. A method for producing the pulp composition according to any one of claims 1 to 10, comprising:
a wax addition of adding the wax to the pulp; and
a paper strength agent addition of adding the paper strength agent to the pulp.
